

## UNITED STATES PATENT OFFICE.

JOHN H. HALL AND MARSHALL F. APGAR, OF HIGH BRIDGE, NEW JERSEY, ASSIGNEES  
TO TAYLOR-WHARTON IRON AND STEEL COMPANY, OF HIGH BRIDGE, NEW JER-  
SEY, A CORPORATION OF NEW JERSEY.

## METHOD OF TREATING MANGANESE-STEEL CASTINGS.

No Drawing.

Application filed June 6, 1922. Serial No. 566,405.

To all whom it may concern:

Be it known that we, JOHN H. HALL and MARSHALL F. APGAR, citizens of the United States, residing at High Bridge, in the county of Hunterdon and State of New Jersey, have invented certain new and useful Improvements in Methods of Treating Manganese-Steel Castings, of which the following is a specification.

10 This invention provides an improved method of treating manganese steel castings of large size and intricate section.

It may be said at the outset that we are aware of Walter Brinton's Patent 812,811, 15 which discloses a method of preparatory treatment of manganese steel before the ultimate toughening treatment. It was the knowledge of and the practice of his invention that enabled us, after years of experimentation, to finally reach a definite conclusion as to the best method of treating large and intricate castings of manganese steel.

Manganese steel in the cast condition, and before treatment, is brittle and is characterized by its high co-efficient of expansion and low thermal conductivity. Hence, in cooling, the heat is radiated so rapidly that the surface becomes cool while the interior is still hot. Contraction occurs contemporaneously with the cooling, which often results in cracked castings. This condition also obtains with thick and thin sections of one and the same casting; and in heating up in the furnace similar conditions arise, and this is 35 one of the faults of the Brinton method of treatment.

In our method of treating castings of large size and intricate section, we remove the casting from the mould while it is still at a red heat and place it in a furnace which is heated to substantially the temperature of the casting. We then seal the furnace, and when the casting and furnace have a temperature in common, we slowly raise the 40 temperature of the casting to about 760° C. and maintain that temperature for a comparatively long or short period according to the size and nature of the casting. The temperature is then slowly reduced in order 45 that all portions of the casting may be cooled at the same rate. When the casting has been brought to a temperature of about 300° C.,

it is removed from the furnace and rapidly cleaned of adhering sand, whereupon it is charged into a furnace of like temperature 55 and heated for the ultimate toughening treatment. The length of our preliminary heating or annealing operation varies from twenty-four hours to five days.

Having described our invention, we 60 claim:

1. The method of treating manganese steel castings of large size and intricate form, which consists in subjecting them to a preliminary annealing, by placing the casting, 65 while still red from the heat of casting, in a furnace having substantially the temperature of the casting, maintaining desirable control so as to establish a uniform temperature as between the casting and the furnace, gradually raising the temperature to 70 about 760° C., and maintaining such temperature for a comparatively long or short period according to the size and nature of 75 the casting.

2. The method of treating manganese steel castings of large size and intricate form, which consists in subjecting them to a preliminary annealing, by placing the casting, 80 while still red from the heat of the casting, in a furnace having substantially the temperature of the casting, maintaining desirable control so as to establish a uniform temperature as between the furnace and the casting, gradually raising the temperature 85 to the requisite maximum annealing temperature, maintaining such temperature for a period determined by the size and nature of the casting, and then slowly reducing the temperature so as to effect the cooling of all 90 portions of the casting at a uniformly slow and regulated rate.

3. The method of treating manganese steel castings of large size and intricate form, 95 which consists in subjecting them to a preliminary annealing, by placing the casting, while still red from the heat of the casting, in a furnace having substantially the temperature of the casting, maintaining desirable control so as to establish a uniform temperature as between the furnace and the casting, gradually raising the temperature 100 to the requisite maximum annealing temperature, maintaining such temperature for

a period determined by the size and nature of the casting, gradually reducing the temperature to about 300° C., and then proceeding in the usual way for the ultimate 5 toughening treatment.

4. The method of treating manganese steel castings of large size and intricate form, which consists in subjecting them to a preliminary annealing by placing the casting, 10 while still red from the heat of the casting, in a furnace having substantially the temperature of the casting, maintaining desirable control so as to establish a uniform temperature as between the furnace and the 15 casting, gradually raising the temperature to about 760° C., holding such temperature for a period determined by the size and nature of the casting, gradually reducing the temperature so as to effect the cooling of 20 all portions of the casting at a uniformly

slow and regulated rate, and then proceeding in the usual way.

5. The method of treating manganese steel castings of large size and intricate form, which consists in placing the casting, while 25 still red from the heat of the casting, in a furnace having substantially the temperature of the casting, sealing the furnace and establishing a uniform temperature as between the furnace and the casting, gradually 30 raising the temperature to about 760° C., holding such temperature for a period determined by the size and nature of the casting, gradually reducing the temperature to about 300° C., rapidly cleaning the casting, 35 and then proceeding in the usual way.

In testimony whereof we affix our signatures.

JOHN H. HALL.  
MARSHALL F. APGAR.